

July 10, 1923.

1,461,643

F. M. BECKET

ALLOY

Filed Nov. 22, 1920



Inventor

Frederick M. Becket,

By *Byers Townsend & Beckenstein*,

Attorneys

## UNITED STATES PATENT OFFICE.

FREDERICK M. BECKET, OF NIAGARA FALLS, NEW YORK, ASSIGNOR TO ELECTRO METALLURGICAL COMPANY, OF NIAGARA FALLS, NEW YORK, A CORPORATION OF WEST VIRGINIA.

## ALLOY.

Application filed November 22, 1920. Serial No. 425,764.

To all whom it may concern:

Be it known that I, FREDERICK M. BECKET, a citizen of the United States, residing at Niagara Falls, in the county of Niagara and State of New York, have invented certain new and useful Improvements in Alloys, of which the following is a specification.

This invention comprises a novel alloy, useful for various purposes, but more particularly in connection with the deoxidation and purification of steel and iron, the production of alloy steels, and the preparation and purification of a wide range of ferrous and non-ferrous metals and alloys, including such alloys as bronzes, stellite, nichrome, etc. The invention comprises also the process involved in the treatment of molten metals or alloys with the said alloy. The alloy contains as its essential components magnesium, silicon and manganese, usually associated with a greater or less proportion of iron.

I have heretofore described an alloy of this general type in my prior Patent 1,222,158, patented November 18, 1919, the said alloy containing magnesium in excess of the equimolecular proportion to the silicon, and preferably in excess of 50% by weight of the alloy. Such alloys are highly efficacious for the purposes set forth in the said patent, but are very energetic in their reaction, which, in certain applications, leads to difficulties in their proper control. The alloys according to the present invention are decidedly less energetic in action and are therefore more readily controlled, and yet they contain the desired amount of magnesium, ranging preferably from 10 to 50% by weight of the alloy.

My investigations have shown that magnesium in material proportions cannot be caused to alloy directly with manganese or iron or mixtures thereof, but that these elements can be caused to alloy with each other by the introduction of a sufficient proportion of silicon. Manganese and iron for the purposes of this investigation are regarded as substantial equivalents. This situation is illustrated by the following typical alloys, in each of which the proportion of manganese (or manganese and iron jointly) is substantially the maximum which it is possible

to cause to enter into the constitution of a homogeneous alloy:

| Per cent.<br>Mg. | Per cent.<br>Si. | Maximum<br>per cent.<br>Mn. | Ratio Si.<br>to Mg. |
|------------------|------------------|-----------------------------|---------------------|
| 10               | 37               | 53                          | 3.7                 |
| 20               | 42               | 38                          | 2.1                 |
| 30               | 43               | 27                          | 1.4                 |
| 40               | 40               | 20                          | 1.0                 |
| 50               | 36               | 14                          | 0.7                 |

As clearly shown by the above table, over the range of 10%-50% magnesium, the ratio of silicon to magnesium varies from 3.7 for 10% magnesium to 0.7 for 50% magnesium, the alloy in each case containing the maximum amount of manganese which it is possible to introduce for a given amount of magnesium. The actual silicon content, however, remains approximately constant over this entire range of magnesium content.

It follows that in the system magnesium-manganese-silicon, at least within the range indicated, there are only a limited number of possible or "real" alloys. This situation is well illustrated in the accompanying drawing, in which the figure is a triaxial diagram, showing the "real" alloys in the unshaded area and the imaginary or non-existent alloys in the shaded area. As stated before iron or mixtures thereof with manganese are practical equivalents of manganese so far as this relation is concerned.

On the basis of the foregoing considerations I have been able to prepare highly efficacious and homogeneous alloys consisting essentially of magnesium, silicon and manganese, together with a greater or lesser proportion of iron. Typical compositions of suitable alloys in accordance with the invention are as follows:

|           |        |        |        |        |
|-----------|--------|--------|--------|--------|
| Magnesium | 4.31%  | 10.20% | 19.29% | 31.01% |
| Manganese | 31.52% | 52.30% | 29.73% | 22.69% |
| Silicon   | 37.14% | 32.10% | 45.30% | 39.84% |
| Iron      | 27.07% | 4.50%  | 2.82%  | 2.51%  |
| Carbon    | 0.03%  | 0.30%  | 0.07%  | 0.17%  |

It will be noted in respect to these several alloys, that the silicon is present in all cases in excess of the equimolecular proportion to the magnesium; and that the manganese, or the manganese and iron jointly, are in lesser molecular proportion than the silicon.

The iron is not regarded as an essential

component of the alloy, but its presence is more or less incidental to the employment of a high grade ferrosilicon as a convenient means of introducing the required amount of silicon into the alloy. In like manner the manganese may be supplied as ferromanganese, with the resulting introduction of further quantities of iron into the alloy.

I claim:-

- 10 1. An alloy containing as essential components magnesium, silicon and manganese, the silicon in excess of the equimolecular proportion to the magnesium, and the manganese in lesser molecular proportion than the silicon.
- 15 2. An alloy consisting essentially of magnesium, silicon, manganese and iron, the silicon in excess of the equimolecular proportion of magnesium, and the manganese and iron jointly in lesser molecular proportion than the silicon.
- 20

3. Process of treating molten metals or alloys for the purification thereof or the production of alloy compositions, which consists in introducing thereinto an alloy containing magnesium, silicon and manganese, the silicon in excess of the equimolecular proportion to the magnesium, and the manganese in lesser molecular proportion than the silicon.

25

4. Process of treating molten metals or alloys for the purification thereof or the production of alloy compositions which consists in introducing thereinto an alloy containing magnesium, silicon, manganese and iron, the silicon in excess of the equimolecular proportion to the magnesium, and the manganese and iron jointly in lesser molecular proportion than the silicon.

30

In testimony whereof, I affix my signature.

FREDERICK M. BECKET.